

## UNITED STATES PATENT OFFICE

2,294,403

## MARKING MATERIAL

Harry W. Helmer and Vinton L. Staley, Chicago,  
Ill., assignors to Helmer-Staley, Inc., Chicago,  
Ill., a corporation of Illinois

No Drawing. Application March 18, 1939,  
Serial No. 262,706

5 Claims. (Cl. 106—19)

This invention relates to solid implements for marking hot surfaces or surfaces to be heated, and more specifically relates to solid marking sticks or pencils composed of a pigment, a vehicle, and a heat-resisting setting agent.

The marking of hot surfaces, or surfaces to be heated such as metal sheets, billets, castings, forgings and the like with identifying data is a troublesome problem in many industries. For example, batches of metal sheets, billets, castings, and the like have a known analysis or designation at the time they are made. Data concerning such analysis or designation, such as a code, color or the like, must be marked on the metal before it has cooled down. Some of the marked metal may then be mixed with metal from other batches and stored for future use. Other metal objects from the same batch may be immediately used or further processed.

The identifying marking on the surface must be clear and permanent enough to withstand handling, weather conditions and the like, and yet not damage the surface by etching the same.

It is sometimes desirable that the marking be removable in pickling baths and the like because, by the time the marked metal objects reach this stage in an industrial process, they are already classified and segregated for a particular use.

We have now provided neutral solid sticks or pencils capable of leaving identifying markings on cold or hot surfaces. The markings will withstand temperatures as high as 1800° F. and will not flake off by mechanical action at any temperature. The marking sticks or pencils of this invention are hard and have appreciable cohesive strength. They are preferably prepared by heating a mixture of the ingredients in powdered form to temperatures to produce a plastic mass. The plastic mass is then extruded through a die into the desired shape. Upon cooling, a hard marking implement of the desired shape is formed.

We have found that solid sticks or pencils capable of marking cold surfaces or surfaces heated as high as 1800° F. can be made from a coloring material or pigment such as Titanox, a solid vehicle therefor, such as halogenated aromatic compounds, and neutral heat-resisting mark-setting agents, such as sodium nitrate, potassium nitrate, sodium sulphate, zinc nitrate, borax and the like, which melt at high temperatures into free flowing liquids having very high boiling points.

In general, the vehicle used should be solid at room temperatures and melt at temperatures below the melting point of the mark-setting

agent. While the vehicle may volatilize or distill off at higher temperatures, the distillation point should be above the melting point of the setting agent. The vehicle is thus active in flowing pigment and setting agent onto hot surfaces at relatively low temperatures. If the surfaces are heated to temperatures above the distillation point of the vehicle, the vehicle will boil off, but, before it leaves the marking, the setting agent will be in a molten condition to anchor the pigment.

We have found that solid halogenated aromatic organic compounds such as chlorinated naphthalenes are excellent vehicles for the pigment as well as bonding agents for the sticks. Chlorinated naphthalenes known commercially as "Halowaxes" are operative.

A Halowax such as tetrachloronaphthalene having a flow point of 270–280° F. and a boiling or distilling range of 680–730° F. has been found with great success. Other Halowaxes, such as hexachloronaphthalene, for example, can be used.

Sodium nitrate, having a melting point of 600° F., is a very satisfactory heat-resisting setting agent for use in combination with the Halowax. It should be noted that the melting point of the sodium nitrate is slightly below the distillation point of the Halowax, so that the setting agent is in a molten condition before the Halowax distills off.

The preferred setting agent should melt to give free-flowing liquids, part of which resist volatilization at the temperatures of the hot surfaces.

It is, then an object of this invention to provide solid marking implements suitable for marking surfaces throughout a wide range of temperatures without damaging the surfaces.

Another object of the invention is to provide neutral solid marking sticks or pencils capable of producing markings on hot surfaces without etching the surfaces.

A further object of the invention is to provide solid marking implements for use in marking hot metal surfaces to leave weather and wear-resisting markings thereon which are readily removed when the metal surfaces are pickled.

A specific object of the invention is to provide a neutral solid marking implement composed of a pigment, a halogenated aromatic organic compound, and an inorganic, heat-resisting setting agent for the pigment.

Another specific object of the invention is to

provide a solid marking implement composed of a pigment, tetrachloronaphthalene, and a neutral inorganic nitrate salt.

Other and further objects of the invention will be apparent from the following examples which illustrate preferred embodiments of the invention:

*Example I*

2 parts by weight of powdered tetrachloronaphthalene are admixed with 2½ parts by weight of powdered Titanox and 2 parts by weight of powdered sodium nitrate. The uniformly mixed powdered mass is then heated to about 130° C. (266° F.) for producing a plastic mass.

The plastic mass is then extruded through a die or mold of the desired diameter to produce an elongated rod. The rod is cut into sticks of the desired length. The sticks are allowed to cool and solidify, and are then ready for packaging.

In the above example the tetrachloronaphthalene content may vary from 1¾ parts to 2½ parts by weight. The sodium nitrate content may be increased to 2½ parts by weight if desired.

The Titanox is a white pigment comprising titanium dioxide together with a filler such as barium sulfate or calcium sulfate and produces a white marking stick leaving a white mark. If desired, coloring materials such as carbon black, iron pigment, cobalt pigment, chromium pigment, and the like can be added to the powdered mixture for producing colored sticks which leave colored markings. Alternatively, other white or colored pigments can be used in place of the Titanox.

*Example II*

2½ parts by weight of a powdered halogenated aromatic organic compound are admixed with 2½ parts by weight of powdered Titanox or other pigment, and 2½ parts by weight of powdered potassium nitrate. The halogenated aromatic organic compound selected should be solid at room temperatures and have a melting point below the melting point of the potassium nitrate.

The uniformly mixed mass is heated to render the same somewhat plastic. The plastic mass is then cast into molds of the desired shape and size. Molding wheels having mating semi-cylindrical notches in their peripheries can be used for the casting operation. The plastic mass is introduced into the nip or bite between the rolls and compressed in the notches of the roll peripheries to form the desired molded article.

After cooling, solid sticks are produced.

The Titanox specified in the above example can be substituted in whole or in part with other pigments or other coloring materials to produce desired shades or colors.

*Example III*

|         | Parts by weight |
|---------|-----------------|
| Borax   | 2               |
| Halowax | 1¾              |
| Pigment | 2½              |

The above ingredients are mixed together to produce a uniformly powdered mass. The powdered mass is then heated to partially fuse the same and the resulting plastic material is molded by extrusion or casting into sticks of the desired size and shape.

Sodium nitrate, potassium nitrate, zinc nitrate, or sodium sulphate can be used in place of the borax in the above example.

10 The marking materials of this invention have considerable cohesive strength and will produce tightly adherent markings on surfaces throughout a wide range of temperatures. Surfaces at 20 temperatures varying from room temperature to 1800° F. can be marked with wear and weather-resisting markings by the marking implements of this invention.

15 It will, of course, be understood that various details of the product and process may be varied 25 through a wide range without departing from the principles of this invention and it is, therefore, not the purpose to limit the patent granted hereon otherwise than necessitated by the scope of the appended claims.

20 We claim:

1. A solid marking implement adapted for the 25 marking of hot metals which comprises a pigment, a neutral meltable solid halogenated aromatic organic compound capable of distilling at elevated temperatures and a neutral heat-resistant 35 pigment-setting agent selected from the group consisting of borax and inorganic nitrate and sulphate salts.

2. A marking stick adapted for marking hot 40 metals which comprises a pigment, a halowax, and an inorganic nitrate salt.

3. A marking stick for marking hot metal surfaces to leave a wear-resisting mark thereon removable in a pickling bath for the metal which 45 comprises a titanium dioxide pigment, tetrachloronaphthalene and sodium nitrate.

4. A solid marking stick for the marking of 50 hot surfaces composed of 1¾ to 2½ parts by weight of tetrachloronaphthalene, 2 to 2½ parts by weight of sodium nitrate and 2½ parts by weight of a titanium dioxide pigment.

5. The method of making marking sticks which 55 comprises uniformly mixing together powdered pigment, powdered tetrachloronaphthalene and powdered sodium nitrate, heating the mixture to about 130° C. to form a plastic mass, extruding the mass into a rod shape, cutting off sticks of desired length from the rod, and allowing the sticks to cool.

HARRY W. HELMER  
VINTON L. STALEY